

# UNITED STATES PATENT OFFICE.

JOHN AUSTIN YATES, OF ROSEBANK, NEW YORK.

## CEMENT AND PROCESS OF MAKING SAME.

No. 833,363.

Specification of Letters Patent.

Patented Oct. 16, 1906.

Application filed January 27, 1906. Serial No. 298,099.

*To all whom it may concern:*

Be it known that I, JOHN AUSTIN YATES, a citizen of the United States of America, residing in the town of Rosebank, county of 5 Richmond, and State of New York, have invented certain new and useful Improvements in Cement and the Process of Making Same, of which the following is a specification.

10 My invention relates to a new and useful composition of matter and to a process for making the same. The new composition is adapted for use as insulating-cement, and particularly for use as the base of an incandescent-light bulb.

15 My composition consists of the following ingredients, combined in the proportions stated: rosin, thirty-two per cent.; zinc oxid, twenty per cent.; marble-flour, forty-eight 20 per cent. These ingredients are ordinary articles of commerce, except that the rosin I prefer to use is that known in commerce as "white" rosin. The cement consisting of the above-named ingredients has been found 25 to combine desired results in the nature of insulating electric wires from each other and in withstanding application of heat up to the point ordinarily met with in service.

20 I now proceed to explain the process of 30 making the cement. By the application of heat I melt the rosin and then add the zinc oxid and bring the mixture to a liquid form, and then add the marble-flour. Of course

during the mixing of the ingredients the matter is thoroughly mingled by agitation. The 35 composition is then applied to where it may be useful and allowed to cool.

What I claim, and desire to secure by Letters Patent, is—

1. A composition of matter consisting of 40 rosin, zinc oxid, and marble-flour.

2. A composition of matter consisting of thirty-two parts of rosin, twenty parts of zinc oxid, and forty-eight parts of marble-flour, combined under the action of heat. 45

3. The process of making cement which consists of reducing rosin to a liquid under the action of heat, mixing zinc oxid therewith and reducing the mixture to a liquid under the action of heat, mixing marble-flour 50 therewith, and allowing the mixture to cool.

4. The process of making cement which consists of reducing thirty-two parts of rosin to a liquid under the action of heat, mixing twenty parts of zinc oxid therewith and reducing the mixture to a liquid under the action of heat, mixing forty-eight parts of marble-flour therewith, and allowing the mixture to cool. 55

In witness whereof I have hereunto set my hand this 26th day of January, 1906.

JOHN AUSTIN YATES.

In presence of—

FRANCIS C. FIELD,  
J. F. BOUDREAU.